

## UNITED STATES PATENT OFFICE

2,506,020

MIXTURE OF INSOLUBLE AMINO-  
ANTHRAQUINONE DYESPaul Grossmann, Binningen, and Walter Kern,  
Sissach, Switzerland, assignors to Ciba Limited,  
a Swiss firmNo Drawing. Application September 14, 1948, Se-  
rial No. 49,292. In Switzerland November 26,  
1947

5 Claims. (Cl. 8—25)

1

It is known that mixtures of dyestuffs are in some cases of advantage for dyeing cellulose esters, for example, artificial silk or staple fibers of lower fatty acids of cellulose, such as cellulose butyrate, cellulose propionate and especially cellulose acetate, and also the corresponding mixed esters. The use of mixtures of dyestuffs is indicated, inter alia, when the dyestuff mixture is required not for producing a desired shade of color but when each of the dyestuffs to be mixed yields dyeings of the same tint or very similar tints, owing to the fact that in many cases such a mixture yields a stronger tint than do the individual pure components of the mixture. This so-called "mixture effect" varies in strength in different instances. It naturally also occurs when by-products are formed in the manufacture of a single dyestuff and the by-products remain in the final dyestuff. Especially pronounced "mixture effects," that is to say those in which the resulting mixed dyeing is very considerably stronger than the dyeings obtainable with the stronger-dyeing component of the mixture, are rare. Moreover, a dyeing of enhanced purity is not to be expected by the use of mixtures, and in some cases, as would be expected, the mixed dyeing is more or less markedly dull.

The present invention is based on the observation that unexpectedly good dyeings on cellulose esters are obtained by using mixtures of which the dyeing constituents consist mainly of 1-( $\beta$ -hydroxyethyl)-amino-4-phenylamino-anthraquinone and 1-methylamino-4-phenylamino-anthraquinone in finely divided form.

As cellulose esters to be dyed by the process of this invention there may be used the known esters of cellulose with aliphatic acids of low molecular weight mentioned above. The fibers of some cellulose ethers and of superpolyamides, superpolyurethanes and superpolyesters are to be regarded as equivalents of fibers of cellulose esters, owing to their similar properties.

The individual components of the mixture, namely 1-( $\beta$ -hydroxyethyl)-amino-4-phenylamino-anthraquinone and 1-methylamino-4-phenylamino-anthraquinone, are in themselves known and can be obtained in various ways. It is of advantage to use them in the present process in a pure or relatively pure state. They may be converted in known manner into a finely divided condition prior to the dyeing process, for example, by grinding with a dispersing agent such as sulfite cellulose waste liquor, advantageously after precipitation, for example, from sulfuric acid.

2

The two components may be mixed together before or during the preparation of the dyebath. The relative proportions of the components may vary within fairly wide limits, but it is of advantage to use not less than 20 per cent., preferably 25-50 per cent., of the component which is present in lower proportion.

Dyeing may be carried out in the usual manner, for example, in aqueous dispersion with the addition of a wetting or dispersing agent such as a soap, an N-benzyl- $\mu$ -heptadecyl-benzimidazole sulfonic acid, a condensation product of taurine or methyl-taurine with a fatty acid, or the like.

It is also of advantage to make a dyestuff preparation which contains the two components mentioned above in the desired relative proportions and in a state of fine dispersion and also contains a wetting or dispersing agent such as sulfite cellulose waste liquor, salts of condensation products from formaldehyde and naphthalene sulfonic acids, naphthenic acid salts, if desired with the addition of wetting agents, such as are mentioned above.

The following examples illustrate the invention, the parts being by weight:

## Example 1

4 parts of 1-( $\beta$ -hydroxyethyl)-amino-4-phenylamino-anthraquinone and 4 parts of 1-methylamino-4-phenylamino-anthraquinone are dissolved in 50 parts of sulfuric acid of 65 per cent. strength. The solution is introduced into a mixture of 160 parts of ice, 240 parts of water and 55 parts of ammonia solution of 25 per cent. strength, stirred well and filtered. The filter residue is washed neutral and ground with about 12 parts of dried sulfite cellulose waste liquor and the necessary quantity of water to form a dyestuff paste containing about 10 per cent. of the dyestuff mixture.

The paste so obtained produces on cellulose acetate artificial silk blue dyeings of great purity. It enables dark blue tints to be obtained which are darker than those obtainable with the individual components of the mixture or can be obtained therewith only by using a very much greater quantity of dyestuff and then not in the same degree of purity.

## Example 2

By using in the procedure of Example 1, 6 parts, instead of 4 parts, of 1-( $\beta$ -hydroxyethyl)-amino-4-phenylamino-anthraquinone and 2 parts, instead of 4 parts, of 1-methylamino-4-phenylamino-anthraquinone, there are obtained similar

results which approach closely the good results obtained in Example 1.

Similar results are obtained by using 2 parts of 1-( $\beta$ -hydroxyethyl)-amino-4-phenylamino-anthraquinone and 6 parts of 1-methylamino-4-phenylamino-anthraquinone.

*Example 3*

10 parts of a paste of 10 per cent strength of finely dispersed 1-( $\beta$ -hydroxyethyl)-amino-4-phenylaminoanthraquinone and 10 parts of a paste of 10 per cent. strength of 1-methylamino-4-phenylamino-anthraquinone are introduced into a solution of 6 parts of the sodium salt of N-benzyl- $\mu$ -heptadecyl-benzimidazole disulfonic acid in 200 parts of water at 30° C., and 3000 parts of water at 40° C. are added while stirring well. 100 parts of well wetted cellulose acetate artificial silk are entered at 40° C., the temperature is raised to 80° C. in the course of  $\frac{1}{2}$  hour, and dyeing is carried on at that temperature for one hour. The artificial silk is then rinsed and finished in the usual manner. A deep blue dyeing is obtained of great purity.

*Example 4*

The procedure is the same as that described in Example 3, except that 20 parts of a dyestuff paste are used containing 10 per cent. of the dyestuff mixture and prepared as described in Example 1 or 2. Very similar results are obtained.

It is to be understood that the amount of dispersing agent contained in the dyestuff preparations is not critical and may range from one tenth to many times the combined weight of the two dyestuffs. The dispersing agent may be omitted altogether if care is taken that, nevertheless, the dyebath prepared with the preparation contains the dyestuffs in finely dispersed condition.

If desired, the dyestuff preparations may be aqueous pastes or thinly liquid dispersions or they may be dried, for example in an atomizer, especially if the amount of dispersing agent is not too low.

It is further to be understood that acetate rayon dyes, other than those specified above, may be present as impurities or purposely added to the preparations in minor amounts, for example if not all of the beneficial effects of the present invention are required, or if the dyes added do not interfere therewith.

What we claim is:

1. A dyestuff preparation in which the dyeing constituent consists mainly of a mixture of 1-( $\beta$ -hydroxyethyl)-amino-4-phenylamino-anthraquinone and 1-methylamino-4-phenylaminoanthraquinone in a finely divided and dispersible condition and in relative proportions ranging from about 4:1 to 1:4, the said anthraquinone compounds being substantially free from impurities possessing affinity for acetate rayon.

2. A dyestuff preparation containing a dispersing agent in which the dyeing constituent consists mainly of a mixture of 1-( $\beta$ -hydroxyethyl)-amino-4-phenylaminoanthraquinone and 1-methyl-amino-4-phenylaminoanthraquinone in a finely divided and dispersible condition and in relative proportions ranging from about 4:1 to 1:4.

3. A dyestuff preparation containing a dispersing agent in which the dyeing constituent consists of a mixture of 1-( $\beta$ -hydroxyethyl)-amino-4-phenylaminoanthraquinone and 1-methyl-amino-4-phenylaminoanthraquinone in a finely divided and dispersible condition and in approximately equal quantities.

4. A dyestuff preparation containing a dispersing agent in which the dyeing constituent consists of a mixture of 1-( $\beta$ -hydroxyethyl)-amino-4-phenylaminoanthraquinone and 1-methyl-amino-4-phenylaminoanthraquinone in a finely divided and dispersible condition and in relative proportions ranging from about 4:1 to 1:4, the said anthraquinone compounds being substantially free from impurities possessing affinity for acetate rayon.

5. A dyestuff preparation consisting of water, a dispersing agent, and approximately equal quantities of 1-( $\beta$ -hydroxyethyl)-amino-4-phenylaminoanthraquinone and 1-methyl-amino-4-phenylaminoanthraquinone in a finely divided and dispersible condition.

PAUL GROSSMANN.  
WALTER KERN.

REFERENCES CITED

The following references are of record in the file of this patent:

UNITED STATES PATENTS

| Number    | Name      | Date          |
|-----------|-----------|---------------|
| 1,967,772 | Grossmann | July 24, 1934 |
| 2,060,136 | Felix     | Nov. 10, 1936 |
| 2,272,294 | Finlayson | Feb. 10, 1942 |
| 2,342,191 | Grossmann | Feb. 22, 1944 |